# EUROPEAN PATENT SPECIFICATION

(11) **EP 1 166 905 B1**
(45) Date of publication and mention of the grant of the patent: **05.10.2005**
(21) Application number: 01202510.2
(22) Date of filing: 29.06.2001
(51) Int. Cl.: B21B 1/22, B21B 3/00

(54) **Method for producing an aluminium sheet and aluminium sheet**
Verfahren zur Herstellung eines Aluminiumbleches und Aluminiumblech
Procédé de fabrication d'une tôle en aluminium et tôle en aluminium

(30) Priority: 29.06.2000 NL 1015568; 11.08.2000 NL 1015921
(43) Date of publication of application: 02.01.2002
(73) Proprietor: Corus Aluminium N.V., 2570 Duffel (BE)
(72) Inventor: Dens, Josephus Maria Théophiel, 2840 Reet (BE); Verboom, Els, 2870 Puurs (BE); Baekelandt, Jean Pierre Jules, 2500 Koninkshooikt (BE); Geibel, Ansgar Maria, 2550 Kontich (BE)
(74) Representative: Hansen, Willem Joseph Maria

(56) References cited:
- EP-A- 0 279 773
- GB-A- 1 017 402
- US-A- 4 634 475
- PATENT ABSTRACTS OF JAPAN vol. 016, no. 217 (M-1252), 21 May 1992 (1992-05-21) -& JP 04 041003 A (FURUKAWA ALUM CO LTD), 12 February 1992 (1992-02-12)
- MARE DE C ET AL: "DEVELOPMENT OF THE SIBETEX SHEET HAVING EXCELLENT DRAWABILITY AND PAINT APPEARANCE" CAHIERS D'INFORMATIONS TECHNIQUES DE LA REVUE DE METALLURGIE, REVUE DE METALLURGIE. PARIS, FR, vol. 94, no. 6, 1 June 1997 (1997-06-01), pages 827-836, XP000701846 ISSN: 0035-1563

## Description

The invention relates to a method for producing an aluminium sheet with a decorative surface structure and to a curved aluminium sheet (see e.g. JP-A 404 1003).

The values which are given in this patent application for surface roughness Ra are all measured in accordance with DIN 4768.

Sheet material, such as for example of aluminium, aluminium alloys and stainless steel, with a decorative surface structure is used, inter alia, for domestic appliances, such as for example the outside of refrigerators and freezers, and for the front panels of audiovisual equipment. Sheet material of this type has a shiny metallic or if desired a matt metallic appearance and, if desired, can be provided with an organic covering layer for further decoration or protection. A typical shiny metallic surface structure is generally obtained by blasting the sheet material with, for example, glass beads or stainless steel shot. One drawback of a surface structure obtained by blasting with beads is that the sheet material is handled in batches and sometimes even by hand, and consequently is rather expensive. Furthermore, it is often the case that an end product, such as for example a refrigerator door, is produced, and then this product is manually or semi-automatically provided with the desired shiny or matt peened surface structure. Moreover, the existing thicknesses for outer sides of domestic materials do not allow, for example, manual blasting with glass beads, on account of the risk of deformation caused by the blasting pressure, and furthermore there is a risk of non-uniformity caused by the manual blasting.

There is a market demand for aluminium sheet material with a surface structure which approximates the surface structure of a glass bead finish as closely as possible. A desired aluminium sheet material of this type must be less expensive than the cost of sheet material with a surface structure obtained by treatment by means of blasting, in particular with glass beads.

It is an object of the invention to provide a method for producing an aluminium sheet with a desired decorative surface structure as described above applied to at least one side of the aluminium sheet.

This problem is solved by the features of claim 1.

The result is a method which can be operated continuously and on an industrial scale to produce aluminium sheet with the desired decorative surface structure described above on at least one side of the aluminium sheet, which decorative surface structure closely to very closely approximates to that of the known finish obtained using glass beads, while the cost price of the finished product is considerably lower than that of aluminium sheet material which is blasted in batches or by hand. A cold-rolled aluminium sheet which is provided typically has a surface roughness Ra in a range from 0.2 to 0.6 microns, measured in accordance with DIN 4768. Furthermore, the method according to the invention ensures that the original mill finish has completely or almost completely disappeared. Mill finish is a term which is known to the person skilled in the art and refers to microscopically visible thin lines oriented substantially in the rolling direction. Furthermore, the method obtained results in a relatively inexpensive semi-finished product on a coil with a desired decorative surface structure, which semi-finished product can then be used to produce end products, such as for example doors for domestic appliances, which then require no further manual treatment.

Although the decorative surface structure of the known finish obtained using glass beads is closely approximated to with a surface roughness of up to Ra 3.0 microns, the roughness Ra which is applied in process step (b) is preferably at most 2.5 microns. Below this value, the decorative surface structure very closely approximates to that of the known finish obtained using glass beads.

It has been found that the appearance of the finish obtained using glass beads is still very closely approximated to in particular with surface roughness values of over Ra 1.8 microns.

In one embodiment of the method according to the invention, the surface roughness is applied to the aluminium sheet by means of rollers with a non-deterministic structure, more preferably by means of electro-discharge texturing rollers, or EDT rollers for short. This allows a desired surface structure to be applied, for example, to a coil of aluminium sheet material continuously and on an industrial scale. Furthermore, the application of the desired surface roughness by means of EDT rollers is achieved, inter alia, through the fact that the original mill finish on the cold-rolled aluminium sheet of the desired final thickness has completely or almost completely disappeared. During the application of the surface structure by means of EDT rollers, the desired result is obtained in one or more light cold-rolling passes. This changes the thickness of the final aluminium sheet by less than 15%, and typically about up to 6%, with respect to the cold-rolled aluminium starting material.

In another embodiment of the method according to the invention, the surface roughness is applied to the aluminium sheet by means of rollers with a non-deterministic structure which are produced with the aid of the precision texturing process. In this process, a small quantity of chromium is applied to the roller in the form of circular or spherical spots.

In an embodiment according to the method, the roller with the non-deterministic structure has a surface roughness Ra in a range between 2 and 6 microns, preferably between 3 and 6 microns, measured in accordance with DIN 4768. Depending on the reduction in the thickness of the aluminium sheet which is employed during the roughening in one or more cold-rolling passes, in this way a desired decorative surface structure within the desired Ra range is achieved on the aluminium sheet.

In one embodiment of the method according to the invention, in a process step (c) the roughened aluminium sheet is provided with a coating layer, for example by means of painting, in which case the coating layer is a layer of paint, or by means of nano-coating, in which case the coating layer is a nano-coating, or by means of anodization, in which case the coating layer is an anodized layer. The nano-coating may comprise a sol-gel process.

The choice of thickness and the type of layer is determined by the end use of the aluminium sheet. Depending on the thickness and the type of layer, the decorative surface structure can be attained or even adapted to the desired appearance of the peened surface structure. Alternatively, the surface can in this way be provided with a desired colour. Moreover, the surface of the roughened aluminium sheet is provided with better protection against scratches and other external influences by the coating layer.

In an embodiment of the method according to the invention, the roughened aluminium sheet is anodized in a process step (c) or is provided with an anodized layer with a thickness in a range of up to 15 microns, more preferably in a range from 3 to 15 microns, by means of anodization. The anodization may be carried out in the customary continuous way on an industrial scale by passing strip material continuously through an anodization bath. Colour anodization is also possible. It has been found that the continuously produced and anodized strip material can also undergo further operations, such as for example punching, bending and light deep-drawing without excessive cracking of the anodized layer which has been applied. Despite the application of a thin anodized layer, the surface roughness applied remains within the given range, and therefore the desired decorative surface structure is also retained. Since it is no longer necessary for a product to be anodized in batches after deformation, there is a considerable reduction in cost of the end product.

Another advantage of anodization over, for example, painting is that the anodized layer obtained by anodization offers very good protection against external chemical influences, such as against spilt cooking ingredients such as tomato sauce and mustard.

In one embodiment of the method according to the invention, the aluminium sheet, after the application of the desired surface roughness and before the anodization, is pickled in a process step (b1). The aluminium sheet may be chemically or electrochemically pickled in an alkaline or acidic medium. More preferably, the aluminium sheet is pickled in an alkaline medium. The intermediate pickling prior to anodization leads to the final sheet material acquiring a surface structure which is somewhat more matt in terms of appearance. For a number of applications of the aluminium sheet obtained using the method according to the invention, this is a highly desirable property of the sheet material. A further advantage is that a pickling treatment is relatively simple to incorporate in a continuous industrial production line which is suitable for the method according to the invention.

In principle, all wrought aluminium alloys which can be treated successfully by means of anodization can be processed in the method according to the invention. However, it has been found that the aluminium alloys which cannot be heat-treated can be processed more successfully than the aluminium alloys which can be heat-treated.

Very good results are obtained with the method according to the invention if an aluminium alloy selected from the Aluminium Association (AA)1xxx series, (AA)3xxx series, (AA)5xxx series and (AA)6xxx series is used for the cold-rolled aluminium sheet. It is preferable to select a wrought aluminium alloy which cannot be heat-treated from the AA5xxx series. These are the aluminium alloys in which magnesium is the most important alloying element. Typical examples which, however, do not limit the invention are the alloys AA5005 and AA5754.

More preferably, the cold-rolled aluminium sheet is brought into a strengthened state, also known as an H temper by the person skilled in the art. This designation applies to products which have been cold-formed after annealing or after hot-forming or to a combination of strengthening and annealing or stabilizing for hardness, in order to obtain the specific mechanical properties. Typical examples which, however, do not limit the invention are an H14 and an H22 temper. It has been found that in particular wrought aluminium alloys with an H temper are very suitable for the application, efficiently and reproducibly on an industrial scale, of the desired surface roughness by cold-rolling, and in particular by EDT rolling.

The invention is also embodied by a curved aluminium sheet part, such as for example the door of a refrigerator or a freezer or the housing of a remote control for audiovisual equipment, produced from an aluminium sheet obtained using the method according to the invention.

The invention will now be explained with reference to a number of examples, which do not restrict the invention.

### Example 1

Aluminium sheet made from the AA5754 alloy in an H temper with a thickness of 0.7 mm on an industrial scale is provided with a surface roughness Ra of 1.35 microns, measured in accordance with DIN 4768, using an industrial EDT roller. The EDT roller used in this example has a surface roughness Ra of approximately 2.5 microns. The roughened aluminium sheet is then pickled lightly in an alkaline solution based on sodium hydroxide, and is then provided, in a sulphuric acid solution, with an anodized layer with a thickness of 5 microns. The final surface roughness Ra of the aluminium sheet obtained was 1.31 microns. The aluminium sheet obtained is then provided with a protective plastic film and was then bent to form a door panel for a refrigerator. The final surface of the door panel provided a very good approximation to the appearance of a finish obtained using glass beads. Gloss measurements were also carried out at an angle of 60°, in accordance with ASTM D-523, on the cold-rolled aluminium sheet after the roughening with the aid of the EDT roller and after the anodization. The results were 175.4 and 25.6 gloss units, respectively.

### Example 2

Aluminium sheet produced from the AA5005 alloy in an H temper with a thickness of 0.5 mm on an industrial scale was provided with a surface roughness Ra of 1.53 microns, measured in accordance with DIN 4768, using an industrial EDT roller. The roughened aluminium sheet was then pickled very lightly in an alkaline solution based on sodium hydroxide and was then provided, in a sulphuric acid solution, with an anodized layer with a thickness of 5 microns. The final surface roughness Ra of the aluminium sheet obtained was 1.52 microns. The aluminium sheet obtained was then provided with a protective plastic film and was then bent to form a panel for a remote control. The final surface of the remote control provided a very close approximation to the appearance of a finish obtained using glass beads. Gloss measurements at an angle of 60° were once again carried out, in accordance with ASTM D-523, on the cold-rolled aluminium sheet after the roughening with the aid of the EDT roller and after the anodization. The results were 182.2 and 23.1 gloss units, respectively.

### Example 3

Aluminium sheet which was produced from the AA5754 alloy in an H temper with a thickness of 0.7 mm on an industrial scale was provided with a surface roughness Ra of 2.1 microns, measured in accordance with DIN 4768, using an industrial EDT roller. The EDT roller used in this example has a surface roughness Ra of approximately 3.8 microns. Then, the roughened aluminium sheet was pickled lightly in an alkaline solution based on sodium hydroxide and was then provided, in a sulphuric acid solution, with an anodized layer with a thickness of 5 microns. The ultimate surface roughness Ra of the aluminium sheet obtained was 2.0 microns. The aluminium sheet obtained was then provided with a protective plastic film and was then bent to form a door panel of a refrigerator. The ultimate surface of the door panel provided a very close approximation to the appearance of a finish obtained using glass beads. Gloss measurements at an angle of 60° were also carried out, in accordance with ASTM D-523, on the cold-rolled aluminium sheet after the roughening with the aid of the EDT roller and after the anodization. The results were 128.3 and 22.7 gloss units, respectively.

For comparison purposes, aluminium sheets were provided with a surface roughness of Ra 0.9 micron and Ra 1.0 micron with the aid of EDT rollers. Visual inspection revealed that these sheets do not have a surface structure which approximates the desired surface structure which would be obtained by blasting with glass beads.

It should be noted that it may be advantageous, in particular for a relatively thick anodized layer and/or substantial deformation operations carried out on the decorative aluminium sheet provided with the decorative surface structure to be curved or bent before the curved aluminium sheet is anodized, despite the higher costs associated with batchwise anodization. This has the advantage that the anodized layer cannot be damaged during the deformation.

## Claims

1. Method for producing an aluminium sheet with a decorative surface structure on at least one side, comprising the successive process steps of:
(a) providing a cold-rolled aluminium sheet of a desired thickness;
(b) using cold-rolling to apply a surface roughness Ra to at least one side of the aluminium sheet, in a range from 1.2 to 3.0 microns measured in accordance with DIN 4768,
**characterized in that** after process step (b) the roughened aluminium sheet surface is provided, in a process step (c), with an anodized layer with a thickness in a range of up to 20 microns by means of anodization.

2. Method according to Claim 1, **characterized in that** said anodized layer has a thickness in a range up to 15µm.

3. Method according to Claim 2, **characterized in that** said anodized layer has a thickness in the range of 3 to 15µm.

4. Method according to Claim 1 to 3, **characterized in that** during process step (b) the surface roughness is applied by means of rollers with a non-deterministic texture.

5. Method according to Claim 4, **characterized in that** during process step (b) the surface roughness is applied by means of electro-discharge texturing (EDT) rollers.

6. Method according to Claims 1 to 5, **characterized in that** after process step (b) and before process step (c) the aluminium sheet is pickled in a process step (b1).

7. Method according to Claim 6, **characterized in that** during the process step (b1) the aluminium sheet is chemically or electrochemically pickled in an alkaline or acidic medium.

8. Method according to one of Claims 1 to 7, **characterized in that** during process step (b) a surface roughness in a range of Ra 1.3 to 3.0 microns is applied, preferably in a range of Ra 1.5 to 3.0 microns, measured in accordance with DIN 4768.

9. Method according to one of Claims 1 to 8, **characterized in that** the roughness Ra which is applied in process step (b) is at most 2.5 microns, measured in accordance with DIN 4768.

10. Method according to claim 1, 2 or 3 **characterized in that** the surface roughness Ra applied in step (b) is over 1.8µm, measured in accordance with DIN 4768.

11. Method according to one of the preceding Claims 1 to 10, **characterized in that** an aluminium alloy from the AA1xxx series, the AA3xxx series, the AA5xxx series or the AA6xxx series is selected for the composition of the aluminium sheet provided.

12. Curved aluminium sheet obtained by the method according to one of Claims 1 to 11, having on at least one side a roughened surface of the aluminum sheet having a surface roughness Ra in the range 1.2 to 3.0 microns measured in accordance with DIN 4768 the curved aluminium sheet further **characterized in** having, on said roughened surface an anodization layer with a thickness in a range of up to 20 microns.

## Patentansprüche

1. Verfahren zur Herstellung eines Aluminiumblechs mit einer dekorativen Oberflächenstruktur auf wenigstens einer Seite, umfassend die aufeinander folgenden Verfahrensschritte des:
(a) Bereitstellens eines kaltgewalzten Aluminiumblechs mit einer gewünschten Dicke;
(b) Anwendens des Kaltwalzens, um eine Oberflächenrauheit Ra auf wenigstens eine Seite des Aluminiumblechs, in einem Bereich von 1,2 bis 3,0 Mikron nach DIN 4768 gemessen, aufzubringen,
**dadurch gekennzeichnet, dass** nach dem Verfahrensschritt (b) die geraute Aluminiumblechoberfläche, in einem Verfahrensschritt (c), mit einer eloxierten Schicht mit einer Dicke im Bereich von bis zu 20 Mikron mittels Eloxierung versehen ist.

2. Verfahren nach Anspruch 1, **dadurch gekennzeichnet, dass** die eloxierte Schicht eine Dicke im Bereich von bis zu 15µm hat.

3. Verfahren nach Anspruch 2, **dadurch gekennzeichnet, dass** die eloxierte Schicht eine Dicke im Bereich von 3 bis 15µm hat.

4. Verfahren nach Anspruch 1 bis 3, **dadurch gekennzeichnet, dass** während des Verfahrensschrittes (b) die Oberflächenrauheit mittels Walzen mit einer nicht deterministischen Struktur aufgebracht wird.

5. Verfahren nach Anspruch 4, **dadurch gekennzeichnet, dass** während des Verfahrensschrittes (b) die Oberflächenrauheit mithilfe von elektroerosiver strukturbildender (EDT) Walzen aufgebracht wird.

6. Verfahren nach Ansprüchen 1 bis 5, **dadurch gekennzeichnet, dass** nach dem Verfahrensschritt (b) und vor dem Verfahrensschritt (c) das Aluminiumblech in einem Verfahrensschritt (b1) gebeizt wird.

7. Verfahren nach Anspruch 6, **dadurch gekennzeichnet, dass** während des Verfahrensschrittes (b1) das Aluminiumblech in einem alkalischen oder sauren Medium chemisch oder elektrochemisch gebeizt wird.

8. Verfahren nach einem der Ansprüche 1 bis 7, **dadurch gekennzeichnet, dass** während des Verfahrensschrittes (b) eine Oberflächenrauheit in einem Bereich von Ra 1,3 bis 3,0 Mikron aufgebracht wird, vorzugsweise in einem Bereich von Ra 1,5 bis 3,0 Mikron, nach DIN 4768 gemessen.

9. Verfahren nach einem der Ansprüche 1 bis 8, **dadurch gekennzeichnet, dass** die Rauheit Ra, die in dem Verfahrensschritt (b) aufgebracht wird, höchstens 2,5 Mikron beträgt, nach DIN 4768 gemessen.

10. Verfahren nach Anspruch 1, 2 oder 3, **dadurch gekennzeichnet, dass** die Oberflächenrauheit Ra, die in dem Schritt (b) aufgebracht wird, über 1,8µm beträgt, nach DIN 4768 gemessen.

11. Verfahren nach einem der vorhergehenden Ansprüche 1 bis 10, **dadurch gekennzeichnet, dass** eine Aluminiumlegierung der AA1xxx-Serie, der AA3xxx-Serie, der AA5xxx-Serie oder der AA6xxx-Serie für die Zusammensetzung des bereitgestellten Aluminiumblechs ausgewählt wird.

12. Gekrümmtes Aluminiumblech, nach dem Verfahren gemäß einem der Ansprüche 1 bis 11 erzielt, das auf wenigstens einer Seite eine geraute Oberfläche des Aluminiumblechs mit einer Oberflächenrauheit Ra im Bereich von 1,2 bis 3,0 Mikron, nach DIN 4768 gemessen, aufweist, wobei das gekrümmte Aluminiumblech des Weiteren **dadurch gekennzeichnet ist, dass** es auf der gerauten Oberfläche eine eloxierte Schicht mit einer Dicke im Bereich von bis zu 20 Mikron hat.

## Revendications

1. Procédé pour fabriquer une tôle d'aluminium à structure de surface décorative sur au moins une face, comprenant les étapes successives d'un processus consistant à :
(a) réaliser une tôle d'aluminium écrouie d'une épaisseur voulue ;
(b) utiliser un laminage à froid pour créer une rugosité de surface Ra sur au moins une face de la tôle d'aluminium, de 1,2 à 3,0 micromètres mesurée conformément à DIN 4768,
**caractérisé en ce que**, après l'étape (b), la surface dépolie de la tôle d'aluminium est dotée par anodisation, lors d'une étape (c) du processus, d'une couche anodisée d'une épaisseur de l'ordre d'un maximum de 20 micromètres.

2. Procédé selon la revendication 1, **caractérisé en ce que** ladite couche anodisée a une épaisseur de l'ordre d'un maximum de 15 µm.

3. Procédé selon la revendication 2, **caractérisé en ce que** ladite couche anodisée a une épaisseur de 3 à 15 µm.

4. Procédé selon la revendication 1 à 3, **caractérisé en ce que**, pendant l'étape (b) du processus, la rugosité de surface est réalisée à l'aide de cylindres à texture non déterministe.

5. Procédé selon la revendication 4, **caractérisé en ce que**, pendant l'étape (b) du processus, la rugosité de surface est réalisée à l'aide de cylindres texturants à électroérosion (TEE).

6. Procédé selon les revendications 1 à 5, **caractérisé en ce que**, après l'étape (b) du processus et avant l'étape (c) du processus, la tôle d'aluminium est décapée lors d'une étape (b1) du processus.

7. Procédé selon la revendication 6, **caractérisé en ce que**, pendant l'étape (b1) du processus, la tôle d'aluminium est décapée par voie chimique ou électrochimique en milieu alcalin ou acide.

8. Procédé selon l'une quelconque des revendications 1 à 7, **caractérisé en ce que**, pendant l'étape (b) du processus, une rugosité de surface Ra de 1,3 à 3,0 micromètres est réalisée, de préférence dans un intervalle de Ra de 1,5 à 3,0 micromètres, mesurée conformément à DIN 4768.

9. Procédé selon l'une quelconque des revendications 1 à 8, **caractérisé en ce que** la rugosité Ra créée lors de l'étape (b) du processus est au maximum de 2,5 micromètres, mesurée conformément à DIN 4768.

10. Procédé selon la revendication 1, 2 ou 3, **caractérisé en ce que** la rugosité de surface Ra créée lors de l'étape (b) est supérieure à 1,8 µm, mesurée conformément à DIN 4768.

11. Procédé selon l'une quelconque des revendications 1 à 10 qui précèdent, **caractérisé en ce qu'**un alliage d'aluminium de la série AA1xxx, de la série AA3xxx, de la série AA5xxx ou de la série AA6xxx est choisi pour la composition de la tôle d'aluminium réalisée.

12. Tôle d'aluminium incurvée réalisée par le procédé selon l'une quelconque des revendications 1 à 11, ayant sur au moins une face une surface dépolie de la tôle d'aluminium à rugosité de surface Ra de 1,2 à 3,0 micromètres mesurée conformément à DIN 4768, la tôle d'aluminium incurvée étant en outre **caractérisée en ce qu'**elle comporte sur ladite surface dépolie une couche d'anodisation d'une épaisseur de l'ordre d'un maximum de 20 micromètres.
